

## UNITED STATES PATENT OFFICE

2,508,857

## METHOD OF RECONDITIONING USED SAND

Marshall V. Chamberlin, Saginaw, Mich., assignor  
to The Dow Chemical Company, Midland,  
Mich., a corporation of Delaware

No Drawing. Application February 15, 1947,  
Serial No. 728,967

4 Claims. (Cl. 22—217)

1

The invention relates to casting light metal, such as magnesium and magnesium-base alloys and aluminum and aluminum-base alloys. It more particularly concerns an improved sand casting method for use with light metals.

In the conventional practice of sand casting light metals, the molds are either of green sand or baked sand and may include one or more baked cores. After the metal is cast, the molds are destroyed, and, in the case of the green sand molds, the sand is ordinarily reused. However, it has not been found feasible with existing methods to reuse the sand of baked molds. This is because the used sand of baked molds is contaminated with the residuum of the binder used in the original molding sand mixture and its presence spoils the permeability and other molding properties of the sand. In order to render such used sand suitable for reuse, the spent binder must be removed and this can be accomplished only by a high temperature calcination or leaching or both. The use of dry or baked sand molds for casting light metals, although highly desirable from the standpoint of making high quality castings, has not been widely used owing to the necessity (with conventional methods) of rejecting the used sand after each casting or applying costly and laborious methods of reclaiming the sand.

The principal object of the invention is to provide a method of casting light metals in which the necessity for either rejecting the used sand or applying costly and laborious reclaiming methods on the used sand are avoided.

Other objects and advantages will appear as the description of the invention proceeds.

My invention is predicated upon the discovery that by forming a molding sand mixture of foundry sand, a reversible organic colloid, such as cereal flour as a binder, and water for tempering, molds made therefrom can be baked to form baked sand molds and then, after the molds have been used for casting light metal, they may be crushed and the crushed molding sand mixture rendered fit for reuse merely by retempering with water and adding, if desirable, a small amount of additional binder and sand to make up for losses. Thus, the sand mixture may be used repeatedly and a succession of high grade castings of light metal may be made with great economy of labor and material.

The invention, then, consists of the method hereinafter fully described and particularly pointed out in the claims.

In carrying out the invention, ordinary foundry sand may be used having a suitable permeability,

2

such as common bank sand, that is free or substantially free from clay. I have found that the presence of clay is undesirable in the sand used in my process. Sufficient water is added to render the sand moldable, i. e. about 2 to 7 per cent of the weight of the sand. A binder of a reversible organic colloid, such as a cereal flour, is added. Various cereals or mixtures of them may be used in flour form. Examples of such binders are corn flour, oat flour, wheat flour, rye flour, and the like. These materials either disperse or dissolve in the water added to the sand to form the binding agent holding the sand grains together during molding and harden when baked, thus strongly cementing the sand grains together thereby giving strength to the mold. All such reversible organic colloids derived from cereals have the property of forming solutions or dispersions in water, and, after being subjected to a drying and baking operation whereby they become hardened, are again capable of being dispersed or dissolved in water. In addition, these materials are somewhat sticky when wet and thus render the sand moldable and when dried adjacent to the sand grains, as in baking the molded sand, cement the sand grains together. These materials are, therefore, capable of being repeatedly alternately rendered sticky by tempering with water and hardened by baking. The proportion of binder used affects the strength of the molded mixture and its permeability to gas and is so chosen as to give the results desired as regards these factors. Generally, the amount to use is in the range of 0.1 to 2 per cent of the weight of the sand. I have found also that a combination of two or more cereal binders are more satisfactory than one cereal. Dextrin, or other equivalent gummy material derived from cereals, when used with the cereal binder, I have found also improves the baked strength of the molded mixture. The term "reversible" is thus used herein to mean the property possessed by the binder of being resoluble or redispersible in water after the water has been baked out of the solution or dispersion.

In addition to the water and binder, it is desirable to employ in the molding sand mixture a relatively small amount of a water-soluble polyhydric alcohol, such as ethylene glycol, glycerine, and the like, as such materials improve the moldability of the sand mixture. A suitable amount is between about 0.1 and 1 per cent of the weight of the sand.

For casting magnesium and its alloys, conventional inhibitors of the oxidation of magnesium may be incorporated in the molding sand mixture.

as in conventional practice. Examples of these agents are: ammonium salts, e. g. NH<sub>4</sub>Cl; fluorides, e. g. NH<sub>4</sub>F, HF; silicofluorides, e. g.



borofluorides, e. g. NH<sub>4</sub>BF<sub>4</sub>; sulfur; and boric acid. Suitable proportions depend upon the agent used and may be between about 0.1 and 4 per cent of the sand weight, although other proportions are sometimes used.

The sand, binder, water, and the other additives, if used, such as oxidation inhibitors and polyhydric alcohol, are intimately and uniformly mixed. The mixture is formed into molds as in the usual foundry operations with light metal. If desired, the cores, if any are used in the mold, may be molded of the same sand mixture.

The molds, and cores if any are made of the sand mixture, are then subjected to a baking operation which sets the binder and thus hardens and strengthens them. Baking is accomplished by heating, preferably in an oven, at a suitable drying temperature above about 212° F. but below the decomposition temperature of the binder, until the binder hardens. To avoid carbonization or decomposition of the binder and loss of oxidation inhibitor if present, the baking temperature should not exceed about 350° F. The time required to harden the molds depends upon their size and may be a few minutes to several hours.

Castings are made in the baked or hardened molds in the usual way, and, after the castings are shaken out of the molds, the used molding sand is reclaimed and made ready for reuse.

Reclaiming is accomplished by sifting the used sand, if necessary so as to remove chills, if any, core wire, etc., and then the bond of baked binder between the sand grains is fractured so that the individual grains are freed and a substantially free-flowing sand is obtained. The bond between the sand grains may be broken by mulling the sand or otherwise subjecting the sand to a pulverizing treatment as by the use of a ball mill which separates the sand grains from each other but does not substantially fracture the grains themselves. The reclaimed used sand is made ready for reuse by retempering with water and other tempering liquid, e. g. polyhydric alcohol, if desired, and incorporating with the sand additional binder, oxidation inhibitor, and some new sand to replenish losses in so far as necessary.

The amount of additional materials needed to replace losses varies according to the nature of the castings produced and is more or less proportional to the ratio of the weight of the casting to that of the sand used for its mold. In general, about 5 to 20 per cent of the binder and about 10 to 40 per cent of the oxidation inhibitor are destroyed during casting and nearly all the tempering liquid is vaporized and lost during baking. Accordingly, appropriate restoration is made when reworking the sand so that an adequate concentration of these materials is present in the sand at the time of molding and casting. In addition, there is always some loss of the sand itself which is carried away with the castings, mold boxes, cores, etc., and as fines and dust in amount up to about 5 to about 25 per cent of the weight of the sand used in each mold and appropriate replacement is made as already indicated. In some instances, higher sand losses may occur as with very complicated castings and those with extremely heavy sections.

The following example is illustrative of a suitable composition for an initial batch of molding sand for use according to the invention:

#### EXAMPLE

|    | Ingredients          | Proportions, Parts by Weight |
|----|----------------------|------------------------------|
| 10 | Sand                 | 100                          |
|    | Oxidation inhibitor: |                              |
|    | Boric acid           | 0.50                         |
|    | Sulfur               | 0.75                         |
| 15 | Binder:              |                              |
|    | Cereal flour         | 0.33                         |
|    | Dextrin              | 0.67                         |
|    | Tempering liquid:    |                              |
|    | Water                | 4.00                         |
|    | Ethylene glycol      | 0.50                         |

The foregoing ingredients are mulled together until thoroughly intermingled, whereby a moldable sand mixture is obtained. This operation usually takes from about 4 to 10 minutes. Table I sets forth pertinent data as regards certain properties of the sand mixture of the above example when formed into a mold and also after baking the mold for 30 minutes at 350° F.

TABLE I

#### Properties of molded new sand mixture

|    |                                            | As Molded | As Baked |
|----|--------------------------------------------|-----------|----------|
| 30 | Permeability <sup>1</sup>                  | 80        | 110      |
|    | Compression Strength <sup>2</sup> p. s. i. | 1.2       | 900      |
|    | Hardness <sup>2</sup>                      |           | 92       |

<sup>1</sup> Determined by the American Foundrymen's Association Standard Method for Determining Permeability.

<sup>2</sup> Dial reading of a standard Dietert core hardness tester.

As already indicated, some of the sand mixture is lost with each casting so that as the sand mixture is recycled, through the operation of molding casting and reclaiming, a certain amount of new sand is added (together with other additives as already explained) at each recycling. As illustrative of this, a succession of test castings were made consisting of a magnesium cylinder about 3 inches in diameter and 12 inches long and weighing about 12.5 pounds, the mold for which required about 85 pounds of the sand mixture having an initial composition as indicated in the example. In these tests, it was found that for each remolding of the sand, new sand was required at the rate of about 25 pounds of new sand for each 75 pounds of used or reclaimed sand; and for each 100 pounds of the mixture of used and new sand about 0.2 part of boric acid, 0.3 part of sulfur, 0.12 part of cereal flour, 0.24 part of dextrin, 0.5 part of ethylene glycol, and 4.0 parts of water were required to restore the molding qualities. The restored molding properties thus obtained are set forth in Table II.

TABLE II

#### Properties of molded reclaimed sand mixture

|    |                                            | As Molded | As Baked |
|----|--------------------------------------------|-----------|----------|
| 65 | Permeability <sup>1</sup>                  | 100       | 110      |
|    | Compression Strength <sup>2</sup> p. s. i. | 1.15      | 950      |
|    | Hardness <sup>2</sup>                      |           | 90       |

<sup>1</sup> Determined by the American Foundrymen's Association Standard Method for Determining Permeability.

<sup>2</sup> Dial reading of a standard Dietert core hardness tester.

Referring to Table II, it is apparent that by the addition of a comparatively small amount of new binder, and inhibitor, and the proper amount of tempering liquid, the molding quality of the sand

is readily restored so that it is substantially the same as, if not better than, that of new sand.

Among the advantages of the invention are that (1) a given batch of sand may be used repeatedly and its volume maintained by the addition of a small proportion of new sand after each molding, thus conserving the use of sand; (2) relatively small amounts of additives suffice to render the sand usable after each casting, thus conserving binder, and inhibitors, if the latter are used; (3) the baked, as well as the unbaked strength of the molds made from the mixture are comparatively high so that handling the molds and casting operations are facilitated; (4) knockout characteristics are good, that is, the molds after use are easily collapsed and the castings can be separated readily from the sand; (5) obnoxious fumes are not produced from the mold when molten metal is cast therein; (6) exceptionally smooth surface castings are obtained which are relatively free from the usual casting defects; (7) in the case of magnesium castings, all the advantages of baked mold casting are obtained together with the added advantage of good protection from oxidation; (8) the problem of the disposal of large quantities of used molding sand is avoided.

I claim:

1. The method of making a succession of castings of a light metal in baked sand molds which comprises mulling together used sand derived from a later step in the method, said used sand containing as used a binder of a heat-hardenable, reversible organic colloid selected from the group consisting of corn flour, oat flour, wheat flour, rye flour, and dextrin and being substantially free from other binders, fresh clean sand to replace losses occurring during the practice of the method, a sufficient amount of a binder of a heat-hardenable, reversible organic colloid selected from the group consisting of corn flour, oat flour, wheat flour, rye flour, and dextrin to render the said fresh sand moldable, and a tempering liquid in amount sufficient to render the resulting mulled mixture moldable; forming molds of the mulled mixture; baking the molds so as to harden the binder, thereby cementing the sand grains together and vaporizing the tempering liquid; casting light metal in the baked molds; separating the castings from the baked molds; and returning the used sand of the baked molds to the aforesaid mulling step.

10

15

20

25

30

35

40

45

50

2. The method according to claim 1 in which a combination of at least two heat-hardenable reversible organic colloidal binders selected from the group consisting of corn flour, oat flour, wheat flour, rye flour, and dextrin is used.

3. The method according to claim 2 in which the combination of at least two heat-hardenable reversible organic colloidal binders includes dextrin.

4. The method of making a succession of castings of magnesium and alloys thereof which comprises mulling together used sand derived from a later step in the method; said used sand containing as used a binder of a cereal flour and dextrin and being substantially free from other binders; fresh clean sand to replace losses occurring during the practice of the method, the amount of said fresh clean sand not exceeding about 35 per cent of the weight of the used sand; about 0.1 to 1.0 per cent of a binder of cereal flour and dextrin based upon the weight of the fresh clean sand; about 0.1 to 1.0 per cent of a polyhydric alcohol, about 2 to 7 per cent of water, and from about 0.1 to 2 per cent of an inhibitor of the oxidation of magnesium, the proportions of the water, alcohol, and inhibitor being based upon the total weight of the sand mixture; forming molds of the mixture; baking the molds so as to harden the binder and vaporize the water and alcohol; casting magnesium or alloy thereof in the so baked molds; separating the castings from the molds and returning the used sand of the molds to the aforesaid mulling step.

MARSHALL V. CHAMBERLIN.

#### REFERENCES CITED

The following references are of record in the file of this patent:

#### UNITED STATES PATENTS

| Number    | Name    | Date          |
|-----------|---------|---------------|
| 1,533,892 | Osborne | Apr. 14, 1925 |
| 1,602,412 | Runyan  | Oct. 12, 1926 |
| 1,700,713 | Campion | Jan. 29, 1929 |
| 2,381,242 | Wood    | Aug. 7, 1945  |
| 2,422,118 | Meyer   | June 10, 1947 |
| 2,444,413 | Weston  | July 6, 1948  |

#### OTHER REFERENCES

The Foundry, May 1943, pages 96, 97 and 183-185.